

## UNITED STATES PATENT OFFICE

GEORGE R. LOCKHART, OF PROVIDENCE, RHODE ISLAND, ASSIGNOR TO MANVILLE JENCKES COMPANY, OF PAWTUCKET, RHODE ISLAND, A CORPORATION OF RHODE ISLAND

## MANUFACTURE OF RAYON

No Drawing.

Application filed April 17, 1929. Serial No. 355,993.

The present invention relates to an improved process for the production of artificial silk or rayon from viscose.

The invention has for its principal object 5 to provide a novel and improved process for desulphurizing and bleaching the viscose in one operation without at the same time forming compounds which will be injurious to the finished material.

10 In the manufacture of rayon by the viscose method, it has been found necessary to subject the unfinished material to a desulphurizing bath to remove certain impurities which consist largely of sulphur and sulphur compounds. The material is then washed and bleached, and is then subjected to further washings and treatments to remove any compounds remaining which may be detrimental to the fibre.

20 In accordance with the process commonly used, the fibre after being wound into skeins is washed and dried and then subjected to the action of a desulphurizing bath which comprises a solution of sodium sulphide and 25 caustic soda or some similar alkaline solution. This solution acts to dissolve out the impurities in the fibre consisting primarily of sulphur or sulphur compounds, either directly or by first changing these impurities 30 into compounds which are soluble. The material is then taken from the desulphurizing bath and washed.

The material is now subjected to the action 35 of a bleaching bath, the bleaching agent being chlorine liquor which acts by the liberation of oxygen to thoroughly bleach the material. Finally, the material is taken from the bleaching bath and is again washed and given certain treatments to remove any 40 excess of alkali or acid or chlorine compounds remaining in or on the fibre.

Up to the present time, it has been considered impossible to desulphurize and bleach the material simultaneously. This is due primarily to the fact that the chlorine liquor solution either directly or indirectly, on account of the action of the liberated oxygen on the free sulphur and sulphur compounds to be found in the material, and also on account of the lime compounds contained in

the chlorine solution, decomposes and combines with impurities in the silk to form hydrochloric, sulphurous and sulphuric acids. These acids are extremely difficult to wash out of the silk and act when the material is dry sooner or later to eat into the fibre so as to make it tender and destroy its utility. In order to prevent this condition, it is therefore usual to desulphurize the silk so far as possible, reducing the sulphur impurities in the material to a minimum before it is subjected to the bleaching operation.

In carrying out the present invention, a method has been provided for combining the processes of desulphurizing and bleaching the viscose in one operation without at the same time forming compounds which will be injurious to the finished material. The applicant has discovered that by the use of 55 hydrogen peroxide in an alkaline bath containing sodium silicate, the processes of desulphurizing and bleaching can be carried out simultaneously, thereby eliminating completely one process in the treatment of the 60 silk.

Apparently, and so far as the applicant can determine, one of the reasons for the success of this method of desulphurizing and bleaching the viscose fibre in one operation is that the hydrogen peroxide is a very active 65 oxidizing agent and gives off great quantities of oxygen very rapidly, particularly when the temperature is raised. This oxygen apparently combines with the free sulphur and sulphur compounds of the fibres to form soluble sulphur salts without any marked tendency towards the formation of sulphurous, sulphuric or other injurious acids. Inasmuch as there is no chlorine liberated either 70 directly or indirectly during the reaction, there is, of course, no tendency towards the 75 formation of hydro-chloric acid. Another 80 reason for the success of the method is apparently that the sodium silicate facilitates the action of the liberated oxygen in forming 85 soluble sulphur salts without the formation of injurious acids, the sodium silicate constituting a reagent capable of reacting with the 90 liberated oxygen and the sulphur and sulphur compounds of the fibre to eliminate 95 100

sulphurous, sulphuric, and other injurious acids and form water soluble salts such as sodium sulphate and sodium thio-sulphate. Apparently also the fact that the bath is of an alkaline character facilitates the formation of the soluble salts and the elimination of sulphurous, sulphuric and other injurious acids. In its broader aspects, therefore, the present invention contemplates the use of 19 oxidizing agents other than hydrogen peroxide, and reagents other than sodium silicate, or baths other than those distinctly alkaline, providing that the reagent or bath is capable of reacting with the liberated 15 oxygen and the sulphur and sulphur compounds of the fibre to eliminate sulphurous, sulphuric, and other injurious acids and form water soluble salts.

The reaction may be further facilitated by 23 the use of sulphonated or pine oil which serves to permit a better penetration of the peroxide into the finer filaments of the silk, and also acts to emulsify any free sulphur remaining and enable it to be washed out 25 readily.

The nature and scope of the invention having been indicated and a manner of practicing the invention having been specifically described, what is claimed is:

26 A process for desulphurizing and bleaching viscose filaments in a single operation which comprises subjecting the said filaments to the action of hydrogen peroxide in an alkaline bath containing additionally sodium silicate.

In testimony whereof I have signed my name to this specification.

GEORGE R. LOCKHART.

46

48

50

55

60

65